

## UNITED STATES PATENT OFFICE

MICHAEL G. CORSON, OF JACKSON HEIGHTS, NEW YORK, ASSIGNOR TO ELECTRO METALLURGICAL COMPANY, A CORPORATION OF WEST VIRGINIA

## ALLOY AND PROCESS OF HEAT TREATMENT

No Drawing.

Application filed November 19, 1926. Serial No. 149,526.

This invention relates to the production of hard and strong alloys containing copper and nickel as the principal constituents. It comprises the addition of silicon in regulated amounts to such alloys to impart to them the ability to assume a hard and strong condition upon suitable heat treatment. The invention also comprises the application of certain processes of heat-treatment to such silicon-containing alloys to bring out the hardening effect of the silicon addition.

In my copending application Serial No. 58,636, filed September 25, 1925, I have disclosed that copper and copper alloys containing regulated minor amounts of one or more of certain silicides, among them nickel silicide,  $\text{Ni}_2\text{Si}$ , will assume a remarkably hard and strong condition if subjected to certain heat treatment. I have also disclosed in the above-mentioned application that nickel may be present in excess of the amount required to combine with the silicon present in the alloy, and that copper-nickel alloys containing as high as 40% nickel can be hardened by heat treatment after a content of silicon has been incorporated. I have now discovered that copper-nickel alloys containing up to 80% and more of nickel and appropriate amounts of silicon are susceptible to hardening when heat-treated as hereinafter described.

My invention is of particular applicability in treating copper-nickel alloys having compositions within the range of those which are known commercially as Monel metal compositions. For example, an alloy containing about 70% nickel and about 3.5% silicon, with the balance principally copper, is hot rolled and then quenched from above 900° C. In the quenched condition the alloy is very soft,—having a hardness of 95 Brinell,—and can be cold worked in any suitable way. The alloy either as quenched or after further working is then subjected to a second heat treatment of the type commercially known as "ageing" or "age-hardening", which comprises holding the alloy at a temperature of from 500° C. to 700° C. for a period of from one hour to twenty-four hours depending upon the temperature at which the heat treat-

ment is carried out. The product is a hard and strong alloy having a complex of desirable properties including a Brinell hardness of 285 and a tensile strength of 145,000 pounds per square inch. The product also shows a reasonable amount of ductility, i. e., 10% elongation in two inches.

It is found that the percentage of silicon required to render the alloy susceptible to hardening by heat treatment varies somewhat with the proportions of nickel and copper. Also the amounts of silicon which can be added without rendering the alloy unworkable vary over a considerable range roughly in proportion to the amount of nickel present in the alloy. To be specific, copper nickel alloys having a nickel content around the lower limit of the range specified, namely 40%, become susceptible to a hardening heat treatment when 1.5% silicon is present and remain fully workable until 4% or more of silicon is added, whereas those alloys having a nickel content of 70% and more become heat hardenable when 2.5% silicon is present and do not become unworkable by rolling or drawing until approximately 10% silicon is added. In the foregoing specific examples, the ratio  $\frac{\text{Ni percentage}}{\text{Si percentage}}$  falls within the range 7 to 28.

While the process of heat treatment has been described with particular reference to its use in treating a specific alloy, it is to be understood that it may be applied to any of the alloys falling within the range outlined. The various factors appertaining to the heat treatment such as temperature and duration of the heat treatment also may vary somewhat from the range above set forth without departing from the invention.

What I claim is:

1. An alloy comprising nickel 40-80%, silicon 1.5-10%, balance principally copper, with the ratio  $\frac{\text{Ni percentage}}{\text{Si percentage}}$  falling within the range 7 to 28.
2. An alloy comprising approximately 70% copper, 10%

nickel, 3.5% silicon, balance principally copper.

3. An alloy comprising approximately 70% nickel, 2.5-10% silicon, balance principally copper.

4. The alloy comprising nickel 40-80%, silicon 1.5-10%, balance principally copper, with the ratio  $\frac{\text{Ni percentage}}{\text{Si percentage}}$  falling within the range 7 to 28, and having such structure, hardness, and other properties as are produced in an alloy of said composition by quenching from a temperature of above 900° C. and ageing at a temperature between 500-700° C.

15 5. An alloy containing approximately 70% nickel, 2.5-10% silicon, balance principally copper, and having such structure, hardness, and other properties as are produced in an 20 alloy of said composition by quenching from a temperature above 900° C. and ageing at a temperature between 500-700° C.

In testimony whereof I affix my signature.  
MICHAEL G. CORSON.

25.

30

35

40

45

50

55

60

65